

Patented Feb. 16, 1943

2,310,981

# UNITED STATES PATENT OFFICE

2,310,981

## REVERSAL PROCESS OF COLOR PHOTOGRAPHY

Emery Meschter, Milltown, N. J., assignor, by  
mesne assignments, to E. I. du Pont de Nemours  
& Company, Wilmington, Del., a corporation of  
Delaware

No Drawing. Application September 19, 1939,  
Serial No. 295,686

7 Claims. (Cl. 95—2)

This invention relates to color photography. More particularly it relates to processes of producing dyed reversed images. Still more particularly it relates to processes of producing superposed dye reversed images in multi-layer film. Still more particularly it relates to the production of superposed dyed reversed images in multi-layer film containing immobile color forming compounds in at least one layer.

This invention has for an object the provision of an improved method of generating dyed reverse images. A further object is to provide dyed reverse images which are of good color density. A further object is to produce simultaneously a plurality of superposed color separation images in multilayer film. A still further object is to produce simultaneously in a multi-layer film blue-green, yellow and magenta dyed images in separate layers representing the color aspect of a scene. Another object is to produce simultaneously in a multilayer film a plurality of reverse dye images, without resorting to re-exposure of any of said layers. Another object is to color develop the middle or buried layer of a multi-layer film containing three superposed differentially sensitized silver halide emulsion layers without re-exposing the said layer. Other objects include the preparation of a more satisfactory color film, a reduction in the number of steps required to process a color film, and a general advance in the art.

The above and other objects are accomplished by the following invention which comprises the use of an aqueous dye forming reducing bath containing an aromatic polyamino developing agent containing at least one unsubstituted amino group and a nitrogenous base free from negative groups and hydroxyl groups attached to carbon atoms.

In a more limited sense the objects are attained by the use of aqueous dye forming reducing baths containing an arylene diamino developing agent and a nitrogenous base free from negative groups and hydroxyl groups attached to carbon, in the presence of a color former capable of forming an indophenol or azomethine dyestuff for developing reversed metal salt images especially silver salt images.

In a still more limited sense, the invention comprises the use of aqueous dye forming reducing baths containing arylene diamino photographic

developing agents containing at least one unsubstituted amino group and preferably free from nuclear hydroxyl groups and a nitrogenous base free from negative groups and hydroxyl groups attached to carbon capable of energizing said developing agent so that it no longer distinguishes between exposed and unexposed silver halides in its reducing action for developing reversed silver salt images in photographic elements.

10 The energizing agents which change aromatic polyamino developing agents containing at least one unsubstituted amino group and especially those free from negative and hydroxyl groups do not fall into any one specific class of bases but fall within numerous classes. The operative nitrogenous bases as previously stated are free from negative groups such as halogen atoms, e. g. Cl, Br; nitro,  $\text{SO}_3\text{M}$ ,  $\text{COOM}$  wherein M is H or a metal, and hydroxyl groups, attached to carbon. 15 The bases which are water soluble or can be readily dispersed in aqueous systems are most effective. Bases which do not have the above constitution, for example, the alkylol amines, e. g. mono-, di- and tri-ethanol amines, do not function in the reducing solutions of the present invention.

20 An important class of nitrogenous bases which are organic amines may be represented by the general formula:



25 wherein each R, R' and R'' may be hydrogen, alkyl, cycloalkyl, aryl, aralkyl, or wherein two R's may represent a divalent polymethylene hydrocarbon or R, R' and R'' together may represent a trivalent hydrocarbon radical such as a polymethenyl radical which, with the nitrogen atom, forms an N-heterocyclic atom.

30 Another important class of compounds which are quaternary ammonium bases may be represented by the general formula:



35 wherein each  $\text{R}_1$ ,  $\text{R}_2$ ,  $\text{R}_3$  and  $\text{R}_4$  may be hydrogen, alkyl, cycloalkyl, aryl, aralkyl, or wherein two

R's may represent a divalent polymethylene hydrocarbon radical or three R's may represent a cyclic trivalent hydrocarbon radical such as a polymethenyl radical which with the nitrogen atom, forms an N-heterocyclic atom.

Another important class of compounds which are aliphatic polyamines may be represented by the general formula:



wherein each R<sub>1</sub>, R<sub>2</sub>, R<sub>3</sub> and R<sub>4</sub> may be hydrogen, alkyl, cycloalkyl, aryl, aralkyl, and further characterized in that the methylene groups may be substituted by alkyl, cycloalkyl, aryl and aralkyl groups and at least one of the methylene groups may be substituted by amino groups, and n is 1 to 8.

As examples of suitable alkyl groups which may be present in each of the above formulae, mention is made of methyl, ethyl, propyl, isopropyl, n-butyl, tertiary butyl, pentyl, isopentyl, octyl, dodecyl, tetradecyl, octadecyl. Suitable cycloalkyl radicals include cyclobutyl, cyclopentyl, and cyclohexyl. Suitable aryl radicals include phenyl, tolyl,  $\alpha$ -naphthyl,  $\beta$ -naphthyl, etc. Among the useful aralkyl radicals may be mentioned benzyl, 2-methyl benzyl, naphthyl-methyl, etc.

The objects are attained in a refinement of the invention by the preparation of reducing compositions, particularly aqueous baths containing an N-dialkyl phenylene diamine of the general formula:



or a water soluble salt thereof, wherein R and R' are the same or different lower alkyl radicals, e. g. methyl and ethyl; and a nitrogenous base free from negative groups and hydroxyl groups and falling within one of the Formulae 1, 2, and 3.

One important embodiment of this invention is concerned with the use of aqueous baths of the above type for the treatment of multi-layer film composed of three superposed differentially sensitized silver halide emulsion layers containing immobile color former compounds which form colors complementary in color to the employed sensitivity range of the respective emulsion layers. This embodiment will be more fully described below.

In another embodiment of the invention the above baths modified by the addition of color formers which are soluble in aqueous solutions or can be readily dispersed therein are used for the development of reversed images, particularly reversed silver halide images in at least one layer of a multi-layer film.

The reversal process of this invention may be used with a wide variety of different types of film structure. The processes, however, all involve the development of a latent image or series of partial latent images corresponding to a scene including colored scenes, in an ordinary non-color-forming photographic developer. The residual silver salts represent a reversed image since they are the counter-part residue of a given amount of silver halide coating, a certain portion

of which has been employed to produce a metallic silver image corresponding to the latent image. The residual silver salts or reversed image can first be freed of the initially developed silver image by means of the well-known bleaching and clearing baths but are preferably directly treated in the dye generating reducing baths described herein in the presence of color formers, especially those capable of forming indophenol or azo-methine dyes.

The reversal processes hereof as previously stated, are of utility in the processing of multi-layer film, including mono- and multipacks composed of differentially color-sensitive photographic emulsion layers. They are of especial utility in processing monopacks comprising at least three differentially color-sensitive silver halide emulsion layers, each containing immobile color formers, which are borne by a transparent base member. One of the layers may be placed on one side of the base and two on the other. The layers may be separated by clear layers, e. g. colloid layers such as gelatin which prevent migration of color formers, sensitizers, which may be dyed to act as temporary filter layers.

A preferred embodiment of the invention involves the reversal processing of multilayer film which is differentially color sensitized and contains light barrier layers and especially treatment of such film wherein the respective color sensitive layers contain a color former which forms upon development a dye complementary in color to the sensitivity of the respective emulsion layer.

Photographic and film elements of the type just described are claimed in Sease and Weber applications, Serial No. 121,904, filed January 22, 1937, now Patent No. 2,191,502, and Serial No. 287,154, filed July 28, 1939. In such films at least one emulsion layer is protected from the action of light after the first development of a reversal process due to the fact that a layer of pre-fogged silver-gelatino-halide emulsion is interposed between at least two differentially color-sensitized emulsion layers.

In order that the invention will be more readily understood a number of reducing baths which can be used for processing film containing color formers will be described. These baths which are of general utility are claimed in copending application of E. Meschter, Serial No. 295,685, entitled "Reducing Baths," filed upon an even date herewith.

#### Bath A

|                           |       |    |
|---------------------------|-------|----|
| p-Amino-N-diethylaniline  | grams | 2  |
| Ammonium hydroxide, conc. | cc    | 25 |
| Sodium sulfite, anhy.     | grams | 2  |
| Water to                  | liter | 1  |

#### Bath B

|                                        |       |    |
|----------------------------------------|-------|----|
| p-Aminodiethylaniline                  | grams | 2  |
| Hexamethylenediamine (55% in methanol) | cc    | 15 |
| Sodium sulfite, anhy.                  | grams | 3  |
| Water to                               | liter | 1  |

#### Bath C

|                           |       |    |
|---------------------------|-------|----|
| p-Aminodiethylaniline     | grams | 3  |
| Ammonium hydroxide, conc. | cc    | 30 |
| Sodium carbonate, anhy.   | grams | 2  |
| Water to                  | liter | 1  |

*Bath D*

|                           |       |    |
|---------------------------|-------|----|
| p-Aminodiethylaniline     | grams | 3  |
| B-dimethylaminoethylamine | cc    | 20 |
| Sodium sulfite, anhy.     | grams | 3  |
| Water to                  | liter | 1  |

*Bath E*

|                       |       |    |
|-----------------------|-------|----|
| p-Aminodiethylaniline | grams | 2  |
| Piperidine            | cc    | 25 |
| Sodium sulfite, anhy. | grams | 2  |
| Water to              | liter | 1  |

*Bath F*

|                                     |       |    |
|-------------------------------------|-------|----|
| 2-amino-5-diethylamino-toluene      | grams | 5  |
| Trimethyl-benzyl-ammonium hydroxide | cc    | 20 |
| Sodium sulfite, anhy.               | grams | 5  |
| Water to                            | liter | 1  |

*Bath G*

|                          |       |    |
|--------------------------|-------|----|
| 4:4-diaminodiphenylamine | grams | 4  |
| Hexamethylenediamine     | do    | 10 |
| Sodium sulfite, anhy.    | do    | 2  |
| Water to                 | liter | 1  |

*Bath H*

|                         |       |    |
|-------------------------|-------|----|
| 1:4-diaminonaphthalene  | grams | 3  |
| Dimethylcyclohexylamine | cc    | 30 |
| Sodium sulfite, anhy.   | grams | 3  |
| Water to                | liter | 1  |

*Bath I*

|                                |       |    |
|--------------------------------|-------|----|
| 4-diethylamino-1-naphthylamine | grams | 5  |
| B-dimethylaminoethylamine      | cc    | 20 |
| Sodium sulfite, anhy.          | grams | 5  |
| Water to                       | liter | 1  |

*Bath J*

|                                                 |       |    |
|-------------------------------------------------|-------|----|
| p-Aminodibutylaniline                           | grams | 3  |
| Hexamethylenediamine (55% solution in methanol) | grams | 20 |
| Sodium sulfite, anhy.                           | do    | 2  |
| Water to                                        | liter | 1  |

*Bath K*

|                                     |       |    |
|-------------------------------------|-------|----|
| p-Aminodiethylaniline               | grams | 3  |
| Trimethyl-benzyl-ammonium hydroxide | cc    | 25 |
| Sodium sulfite, anhy.               | grams | 3  |

Water to

1

The following examples are directed to various processes involving the reduction of a silver salt image to metallic silver with the use of color-formers in emulsions. It is to be distinctly understood that the following examples are merely illustrative of the nature of the invention and are not intended to limit it in any way.

*Example I*

A monopack comprising a cellulose acetate film base suitably subbed is coated with a gelatin silver bromide emulsion sensitized to red so as to exhibit very little sensitivity in the green spectral region by means of a green blind sensitizing dye, e. g. pinacyanol. To this blue-red sensitive emulsion layer is added 15 grams of a non-migratory blue-green color-former, e. g. a salicylaldehyde-o-sulfobenzaldehyde acetal of polyvinyl alcohol per 1,000 grams of emulsion. Over this blue-red sensitive layer is coated another silver halide emulsion layer which is sensitized to the blue-green region of the spectrum with a sensitizing dye, e. g. erythrosin, and contains a magenta (minus green) color former, e. g. 1-(m-stearoylaminophenyl)-3-methyl-5-pyrazolone. 75

Over the last-mentioned layer is coated a layer of gelatin solution containing a removable yellow filter dye, e. g. Tartrazine C. I. 640. Over the yellow filter layer is coated a blue sensitive silver halide emulsion containing a yellow color former, e. g. furoyl-acetbenzoylacet-benzidide.

The above-described film element is exposed to a colored object scene whereby latent images representing different color component aspects in the different sensitive layers are formed as is known in the art. See, for instance, Schinzel Austrian Patent No. 42,478. The film is then processed by the following steps:

1. Develop 10 minutes in an ordinary metol-hydroquinone positive developer.

2. Wash 10 minutes.

3. Reduce residual silver salts by treating for 15 minutes in a dye-generating reducer of the following formula:

Sodium sulfite, anhydrous grams 1.0

p-aminodiethyl aniline dihydrochloride grams 2.0

Hexamethylene diamine (40% solution) cc 20

Water to liter 1

4. Wash 10 minutes.

5. Bleach 7 minutes in a solution containing 3 1/2% by weight of potassium ferricyanide and made alkaline with ammonium hydroxide or sodium carbonate.

6. Rinse.

7. Remove bleached silver in a 25% solution of hypo (crystalline sodium thiosulfate).

8. Wash 15 minutes and dry.

The color photograph resulting from the above process is of exceptional clarity and brilliancy. The saturation of dyes or dye densities is considerably greater than that obtained by known methods of processing. The images have very good resistance to fading, particularly under action of ultra violet radiation.

*Example II*

45 A cellulose acetate film base is coated with a 30 mg. coating of a silver bromide emulsion sensitized to the red region of the spectrum with a green-blind, red sensitizing dye, e. g. a naphthiocarbocyanine, containing a blue-green color former of the type set forth in Example I. Over this layer is coated a 25 mg. coating of silver bromide which was precipitated in the presence of 1/2 the normal amount of gelation with about 0.5 gram of allyl thiourea per kilogram of final emulsion, said emulsion being digested for one hour at 120° F. and the remaining gelatin added and dissolved. Over the pre-fogged layer is applied a 35 mg. orthochromatized silver bromide emulsion containing 5 grams of the magenta color-former of Example I. Another coating of pre-fogged emulsion containing a yellow (minus blue) filtering material, e. g. 6 grams of titanium ferrocyanide or 4 grams of 4-piperonylbutadienyl-a-pyridinium stearyl bromide, was superposed on said orthochromatized layer. Over this pre-fogged filter layer is coated a 38 mg. coating of blue sensitive high contrast silver chloro-bromide emulsion containing about 8 grams of a yellow color former, e. g. dibenzoylacetbenzidide.

The just described multilayer film is exposed to a colored scene which may be from an optical image or the image produced from a color transparency according to the steps of reversal process set forth in Example I, using, however, in

place of the reducer described in Step 3, the following reducer:

|                                        |       |    |
|----------------------------------------|-------|----|
| Sodium sulfite, anhydrous              | grams | 5  |
| p-Aminodiethyl aniline dihydrochloride | grams | 4  |
| Sodium carbonate, anhy.                | do    | 20 |
| Ammonium hydroxide, conc.              | cc    | 30 |
| Water to                               | liter | 1  |

The resulting film was of exceptional clarity 10 and brilliancy and the dye images of good density.

In place of the specific dye-forming reducing baths of the preceding examples may be substituted a wide variety of reducing baths having the above-described characteristics. Thus, any 15 of the baths described in the aforescribed application may be substituted with similar result.

Similarly, various other immobile color formers, may be substituted for the specific color formers set forth in the above examples. Color formers which give excellent results include non-migratory yellow color-formers, which may be used in the blue-sensitive layer, as follows: diacyacetamino-aryl-bis-thiazoles of U. S. Patent 2,140,540, of which difuroylacetamino-1,2,4,5-benzo-bis-thiazole and di-acetoacetamino-1,2,4,5-benzobisthiazole are especially useful as are 2-hydroxy-3-naphthoylaminobenzoyl-acetanilide, sodium stearoylamino-benzoylacetanilide-p-carboxylate, p-caproylamino-, benzoylamino-salicylic acid, furoylacet-p-amino phenyl-amyl ether (described in Jennings and Middleton application, Serial No. 215,702, filed June 24, 1938, now Patent No. 2,184,303), and di-picolinoyl-acet benzidine.

Suitable non-migratory magenta color-formers which are especially useful are 1-(3'-sulfophenyl)-3-(4'-stearoylamino phenyl)-3-(4'-dodecoylamino-phenyl)-5-pyrazolone, 4,4'-bis-(3'-methyl pyrazolonyl-1')-diphenyl (described in Jennings & Middleton, Serial No. 215,703, filed June 24, 1938, now Patent No. 2,200,924), 4,4'-methylene-bis-(m-stearoylaminophenyl)-methyl pyrazolone (described in Jennings, Serial No. 256,201, filed February 13, 1939), and 4,4'-o-sulfo-benzylidene-bis-(phenyl methyl pyrazolone) (described in Jennings, Serial No. 256,201, filed February 13, 1939).

Suitable non-migratory blue-green color formers of especial utility include 4,4'-di-(1-hydroxy-2-naphthoyl-amino) diphenyl, 1-hydroxy-2-carboxy-5-dodecoylamino naphthalene, 1-N-stearoyl-4-N-(1'-oxy-2'-naphthoyl)-phenylenediamine sodium sulfonate, resorcinol mono-n-decyl ether (described in Salzberg & White U. S. Patent No. 2,166,181 (filed September 21, 1937), product of p-hydroxybenzoic acid and formaldehyde (described in McQueen, Serial No. 261,794, filed March 14, 1939), product of polyvinyl alcohol and salicyaldehyde (described in Dorough & McQueen, Serial No. 233,480, filed October 5, 1938).

### Example III

A multilayer film so disposed that light after passing through an optical aperture is first incident on a blue-sensitive silver halide emulsion containing a yellow filter dye such as Luxol Fast Yellow T, then a pre-fogged emulsion layer, then a green sensitive emulsion, another pre-fogged emulsion layer containing a soluble red dye, e. g. carmosine M, then a red sensitive silver halide emulsion, and finally the base. The amount of silver salt in the pre-fogged layers and the fogging exposure given the layers is such that upon

the first development of the layers a light barrier layer will be formed therein so that substantially less than 1% of light will be transmitted by either of them.

In using this film, it is exposed normally in a camera, and then developed in a non-color-forming developer. After development and washing the film contains three color separation negative image layers bearing both silver and unexposed, undeveloped, silver-salt images, and two layers of metallic silver. The film is now preferably exposed through the base with a red or white printing light which exposes only the silver salt image remaining in the red sensitive layer. The red light does not substantially effect the other two layers because of their lack of sensitivity to the red light used as the printing light, and secondly, the black metallic silver barrier layer prevents substantially all of the printing light from passing through to the outer layers.

The film is now developed in a dye forming reducing bath of the following composition:

|                                    |       |    |
|------------------------------------|-------|----|
| 2:3:4-trichlor- $\alpha$ -naphthol | grams | 2  |
| 2-amino-5-diethylaminotoluene      | do    | 5  |
| Potassium carbonate                | ccs   | 10 |
| Sodium sulfite, anhy.              | grams | 5  |
| Water to                           | liter | 1  |

prepared by dissolving the trichloronaphthol in alcohol and adding the other ingredients to water and bringing the solution up to one liter, whereby a blue-green (minus-yellow) dye image and silver image is formed. The film is then thoroughly washed.

The top or blue sensitive layer is then exposed to a blue or preferably a white printing light. This printing light does not affect the middle layer because of the metallic silver barrier layer between the top and middle layers. The entire film is then treated with a yellow (minus-blue) color-forming developer of the following composition:

|                                      |       |    |
|--------------------------------------|-------|----|
| Potassium carbonate                  | grams | 40 |
| Sodium sulfite, anhy.                | do    | 5  |
| Diethyl-paraphenylene diamine hydro- |       |    |
| chloride                             | do    | 3  |
| Water to                             | liter | 1  |

to which is added the following solution:

|                 |                                |
|-----------------|--------------------------------|
| Benzoyl acetone | 3 grams dissolved in 25 cc. of |
|                 | ethyl alcohol.                 |

After development, the blue-sensitive layer will contain both metallic silver and yellow dye images. It is then thoroughly washed.

The green-sensitive middle layer or both sides of which are black, metallic silver barrier layers, remains. This layer is treated in a dye-forming reducing bath of the type herein described containing an arylene diamino compound and a nitrogenous base and a magenta color former. A suitable bath is composed of

|                                  |       |    |
|----------------------------------|-------|----|
| Thioindoxyl-carboxylic acid      | grams | 2  |
| p-Amino-N-diethylaniline         | do    | 3  |
| $\beta$ -Dimethylaminoethylamine | cc    | 20 |
| Sodium sulfite, anhy.            | grams | 3  |
| Water to                         | liter | 1  |

### Example IV

A multilayer film comprising a transparent support coated on one side first with a 35 mg. coating of fogged silver-gelatino-bromide emulsion and a layer of orthochromatized emulsion is coated on the fogged emulsion layer. On the other side of the support is coated first a 30 mg. layer 70 of silver bromide emulsion, sensitized to the red

region but not to the green region, and containing an immobilized blue-green indo-phenol-forming dye component and over this is coated a 30 mg. layer of blue-sensitized silver chloride emulsion dyed with Tartrazine, C. I. 640.

After exposure to a natural colored scene, the above film is developed in an ordinary metol-hydroquinone developer of the type usually employed for positive film development and then washed. The following processing stages are then given the film:

1. The orthochromatized layer is flashed with white light, through the base.
2. Film is developed in

|                                  |       |    |
|----------------------------------|-------|----|
| Sodium sulfite, anhy.            | grams | 5  |
| 2-Amino-5-N-diethylamino-toluene | do    | 5  |
| Sodium carbonate, anhy.          | do    | 25 |
| Water to                         | liter | 1  |

to which add:

|                                     |       |   |
|-------------------------------------|-------|---|
| 4:4'-bis-(3"-methylpyrazolonyl-1")- |       |   |
| biphenyl                            | grams | 3 |

3. Wash.

4. Flash blue-sensitive layer.

5. Develop in:

|                               |       |    |
|-------------------------------|-------|----|
| Sodium carbonate, anhydrous   | grams | 30 |
| Sodium sulfite                | do    | 5  |
| p-Amino-N-diethylaniline, HCl | do    | 3  |
| Water to                      | liter | 1  |

to which is added the following solution:

Benzoylacet-p-amino-N-phenyl-morpholine, 3 grams dissolved in 25 cc. of ethyl alcohol

6. Wash.
7. Immerse film in one of reducers described under baths A to K.
8. Wash.
9. Bleach in alkaline potassium ferricyanide solution.
10. Wash.
11. Fix in plain, 25%, hypo solution.
12. Wash and dry.

The film and process described above offers the advantages:

A. It affords a possibility of controlling the exposure, and therefore, dye-density characteristics of two outer layers.

B. The middle or "buried" layer is not processed by a developer, partially exhausted from having first developed an upper layer.

C. The middle or "buried" layer receives most energetic reduction, therefore outside layers can be flashed accordingly heavy.

The energetically working reducer applied to reduce the middle or buried layer will also probably reduce silver halides in the other layers which were not developed by the color-forming developers, however, since only the buried layer contains a color-former, no additional color is formed in the outside layers. The additional silver reduced in the outside layers is removed along with the silver images in the ferricyanide-hypo treatment.

#### Example V

A photographic support, which may be a transparent film or a paper base and suitably subbed, is coated with a 30 mg. layer of silver bromide emulsion, sensitized in the red but not the green regions, and containing 30 grams of salicyl-aldehyde-phthalaldehydic acid acetal of poly-vinyl alcohol per kilogram of emulsion. Over this is coated a thin separator layer of plain

gelatin and on this is applied a 35 mg. layer of silver bromide emulsion sensitized into the green region and containing 24 grams 1-(m-stearoyl-amino-phenyl)-3-methyl-5-pyrazolone per kilogram of emulsion. Over the green sensitive layer is coated another thin separator layer of plain gelatin and over this is coated a gelatin layer containing a yellow screening dye such as Tartrazine O, C. I. 640 or 4-piperonylbutadienyl-alpha-pyridinium-stearyl bromide. Over the yellow filter layer is applied a 25 mg. coating of chloro-bromide emulsion containing 20 grams of dibenzoyl acet-benzidine.

After exposure to a colored scene, the above film is processed as in Example I. The color-generating reducing bath for this film is that given as Bath C in the series of energized reducing baths listed above.

#### Example VI

The dye-generating reducing baths of the present invention are particularly suited for the mass production of color photographs on paper by the use of multilayer stripping films, the individual layers of which contain indophenol, azomethine and azo dye-forming components. Such films are fully described in copending Marasco application, Serial No. 245,274, entitled "Photographic films," now Patent No. 2,182,184. A preferred form of color stripping paper can be prepared by coating a double-weight, photographic paper support with an acid-stripping layer from the following solution:

|                           | Grams |
|---------------------------|-------|
| 35 Piperidylmethylzein    | 4.0   |
| Chrome alum               | 0.2   |
| Acetic acid (glacial)     | 4.75  |
| Ethyl alcohol (65% water) | 91.0  |

On this is applied a thin coating of ethyl cellulose dope:

|                 | Grams |
|-----------------|-------|
| Ethyl cellulose | 5.0   |
| Methyl acetate  | 77.0  |
| Acetone         | 11.7  |
| Xylene          | 6.3   |

This thin film support is suitably subbed and then coated with a layer of silver chloro-bromide emulsion sensitized in the red but not in the green region. Red sensitizing dyes which give absolutely no sensitizing action in the green region are described in Middleton and Jennings co-pending application, Ser. No. 174,114, now Patent No. 2,270,378. This green-blind, red sensitive layer contains approximately 20 grams of octadecyl ether of resorcinol per kilogram of emulsion as the blue-green color-forming compound. On the red sensitive emulsion layer is coated another thin film layer of ethyl cellulose, suitably subbed and then coated with a subbing layer and then a coating of green sensitized silver chloro-bromide emulsion containing 4:4'-bis-(3"-methyl-pyrazolonyl-1")-biphenol.

Another acid stripping layer of piperidylmethyl zein is applied over the green sensitive layer, followed by a thin ethyl cellulose coating which is then subbed to receive a blue sensitive silver-chloride emulsion containing Tartrazine O as the yellow filter dye and dibenzoylacetbenzidine as the yellow color-forming material.

The above multilayer color stripping film is printed by exposing through a colored positive transparency, which is preferably of the color-line or color-grain type, with a printing light suitably filtered so that it transmits three sharp-

ly defined color-bands each within the corresponding transmission band of the color element of the color screen. After exposure, the stripping film is developed in a contrasty Metol-hydroquinone developer, washed, reversed in a sulfamic acid-dichromate bleach bath as described in McQueen co-pending application, Serial No. 233,117, now Patent No. 2,195,149, cleared in a 5% sodium sulfite solution, and washed. The combined stripping films lose their anchorage during the bleaching operation and are then stripped off and transferred to temporary supports, such as glass plates. The residual silver salt images remaining in each of the three layers are then reduced to metallic silver by means of one of the baths listed under A to K with the concomitant formation of respective dye images and the silver images are removed as previously indicated. The stripped layers are then superposed in register on a suitable white paper support. The advantages offered by the present process over previous methods is the control of dye-density and dye-gamma values afforded by controlling the time of treatment by the dye-generating reducing baths. Since the increase in dye-density with these reducers continues over a much longer period of time than with ordinary color-developers, the resulting dye-gamma values can be varied over a wide range, thus affording the opportunity to prepare color-prints of time chromatic rendition.

The energetic action of the dye-generating reducers described previously provides an improved means for processing the sound record areas of films for the production of colored sound films. An exemplary procedure appears below.

In the normal arrangement of sensitized emulsion layers and color-forming compounds, and particularly with the introduction of sound recording systems employing ultra-violet radiation as the recording radiation, the sound record is placed in the upper portion of the uppermost emulsion layer and, under ordinary processing methods, would finally appear as a yellow sound track. With the spectral response of photoelectric tubes and the dye-gamma characteristics of yellow color-forming compounds as they are, it is desirable to process the sound area to blue or black rather than yellow.

#### Example VII

Using a multilayer film as described in Example V, the film is exposed so as to contain supplemental latent images in the various emulsion layers and the latent sound record image in the uppermost layer, by layer-localized printing from master separation positive records and ultra-violet printing of the sound record.

The picture-and-sound film is then processed by first covering only the sound area with a water-proof lacquer, a suitable coating composition for which is:

|                                                                                                                                                                                                                                                                                                                                                                                                                                                                                                                                                                                                                                                                                                                                                                                                                                                                                                                                                                                                                                                                                                                                                                                                                                                                                                                                | Per cent<br>by weight |
|--------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|-----------------------|
| Ethyl cellulose (ethoxy content 2.50 mols/C <sub>6</sub> H <sub>5</sub> )                                                                                                                                                                                                                                                                                                                                                                                                                                                                                                                                                                                                                                                                                                                                                                                                                                                                                                                                                                                                                                                                                                                                                                                                                                                      | 1.8                   |
| unit                                                                                                                                                                                                                                                                                                                                                                                                                                                                                                                                                                                                                                                                                                                                                                                                                                                                                                                                                                                                                                                                                                                                                                                                                                                                                                                           | 98.2                  |
| Ethyl alcohol                                                                                                                                                                                                                                                                                                                                                                                                                                                                                                                                                                                                                                                                                                                                                                                                                                                                                                                                                                                                                                                                                                                                                                                                                                                                                                                  |                       |
| This protective layer dries rapidly and the film is then processed as follows:                                                                                                                                                                                                                                                                                                                                                                                                                                                                                                                                                                                                                                                                                                                                                                                                                                                                                                                                                                                                                                                                                                                                                                                                                                                 |                       |
| 1. Develop 8 minutes in contrasty metol-hydroquinone developer (shown on page 5, col. 1, of specification).                                                                                                                                                                                                                                                                                                                                                                                                                                                                                                                                                                                                                                                                                                                                                                                                                                                                                                                                                                                                                                                                                                                                                                                                                    |                       |
| 2. Wash.                                                                                                                                                                                                                                                                                                                                                                                                                                                                                                                                                                                                                                                                                                                                                                                                                                                                                                                                                                                                                                                                                                                                                                                                                                                                                                                       |                       |
| 3. Reduce residual picture silver halides with dye-forming reducing bath D.                                                                                                                                                                                                                                                                                                                                                                                                                                                                                                                                                                                                                                                                                                                                                                                                                                                                                                                                                                                                                                                                                                                                                                                                                                                    |                       |
| 4. Wash and blow-off surface water.                                                                                                                                                                                                                                                                                                                                                                                                                                                                                                                                                                                                                                                                                                                                                                                                                                                                                                                                                                                                                                                                                                                                                                                                                                                                                            |                       |
| 5. Bathe in 95% ethanol to remove protective ethyl cellulose coating.                                                                                                                                                                                                                                                                                                                                                                                                                                                                                                                                                                                                                                                                                                                                                                                                                                                                                                                                                                                                                                                                                                                                                                                                                                                          |                       |
| 6. Develop sound track in metol-hydroquinone developer.                                                                                                                                                                                                                                                                                                                                                                                                                                                                                                                                                                                                                                                                                                                                                                                                                                                                                                                                                                                                                                                                                                                                                                                                                                                                        |                       |
| 7. Wash.                                                                                                                                                                                                                                                                                                                                                                                                                                                                                                                                                                                                                                                                                                                                                                                                                                                                                                                                                                                                                                                                                                                                                                                                                                                                                                                       |                       |
| 8. Reduce residual sound area silver halides with bath K in which has been dissolved 5 grams of a-naphthol.                                                                                                                                                                                                                                                                                                                                                                                                                                                                                                                                                                                                                                                                                                                                                                                                                                                                                                                                                                                                                                                                                                                                                                                                                    |                       |
| 9. Wash.                                                                                                                                                                                                                                                                                                                                                                                                                                                                                                                                                                                                                                                                                                                                                                                                                                                                                                                                                                                                                                                                                                                                                                                                                                                                                                                       |                       |
| 10. Bleach and remove silver images.                                                                                                                                                                                                                                                                                                                                                                                                                                                                                                                                                                                                                                                                                                                                                                                                                                                                                                                                                                                                                                                                                                                                                                                                                                                                                           |                       |
| 11. Wash and dry.                                                                                                                                                                                                                                                                                                                                                                                                                                                                                                                                                                                                                                                                                                                                                                                                                                                                                                                                                                                                                                                                                                                                                                                                                                                                                                              |                       |
| 15. By the above method it is possible to produce continuous lengths of cinematographic bearing natural color picture images and single-color sound records in continuous processing machines of extreme simplicity and economy of operation.                                                                                                                                                                                                                                                                                                                                                                                                                                                                                                                                                                                                                                                                                                                                                                                                                                                                                                                                                                                                                                                                                  |                       |
| 20. In place of the aromatic polyamines free from nuclear hydroxyl groups set forth in the above examples, may be substituted in whole or in part one or more other specific compounds. Suitable additional compounds of this type, which are known photographic developing agents include:                                                                                                                                                                                                                                                                                                                                                                                                                                                                                                                                                                                                                                                                                                                                                                                                                                                                                                                                                                                                                                    |                       |
| 25. 1:4-diaminobenzene                                                                                                                                                                                                                                                                                                                                                                                                                                                                                                                                                                                                                                                                                                                                                                                                                                                                                                                                                                                                                                                                                                                                                                                                                                                                                                         |                       |
| 2:5-diaminotoluene                                                                                                                                                                                                                                                                                                                                                                                                                                                                                                                                                                                                                                                                                                                                                                                                                                                                                                                                                                                                                                                                                                                                                                                                                                                                                                             |                       |
| p-Aminomethyl aniline                                                                                                                                                                                                                                                                                                                                                                                                                                                                                                                                                                                                                                                                                                                                                                                                                                                                                                                                                                                                                                                                                                                                                                                                                                                                                                          |                       |
| p-Aminoethyl aniline                                                                                                                                                                                                                                                                                                                                                                                                                                                                                                                                                                                                                                                                                                                                                                                                                                                                                                                                                                                                                                                                                                                                                                                                                                                                                                           |                       |
| p-Aminodimethyl aniline                                                                                                                                                                                                                                                                                                                                                                                                                                                                                                                                                                                                                                                                                                                                                                                                                                                                                                                                                                                                                                                                                                                                                                                                                                                                                                        |                       |
| p-Aminodiethyl aniline                                                                                                                                                                                                                                                                                                                                                                                                                                                                                                                                                                                                                                                                                                                                                                                                                                                                                                                                                                                                                                                                                                                                                                                                                                                                                                         |                       |
| p-Aminodibutyl aniline                                                                                                                                                                                                                                                                                                                                                                                                                                                                                                                                                                                                                                                                                                                                                                                                                                                                                                                                                                                                                                                                                                                                                                                                                                                                                                         |                       |
| 2-amino-5-diethylaminotoluene                                                                                                                                                                                                                                                                                                                                                                                                                                                                                                                                                                                                                                                                                                                                                                                                                                                                                                                                                                                                                                                                                                                                                                                                                                                                                                  |                       |
| 2:5-diaminomethoxybenzene                                                                                                                                                                                                                                                                                                                                                                                                                                                                                                                                                                                                                                                                                                                                                                                                                                                                                                                                                                                                                                                                                                                                                                                                                                                                                                      |                       |
| 1-amino-4-phenylaminoacetic acid                                                                                                                                                                                                                                                                                                                                                                                                                                                                                                                                                                                                                                                                                                                                                                                                                                                                                                                                                                                                                                                                                                                                                                                                                                                                                               |                       |
| 4:4'-diaminodiphenylamine                                                                                                                                                                                                                                                                                                                                                                                                                                                                                                                                                                                                                                                                                                                                                                                                                                                                                                                                                                                                                                                                                                                                                                                                                                                                                                      |                       |
| 2:4-diaminodiphenylamine                                                                                                                                                                                                                                                                                                                                                                                                                                                                                                                                                                                                                                                                                                                                                                                                                                                                                                                                                                                                                                                                                                                                                                                                                                                                                                       |                       |
| 4-amino-N-phenylpiperidine                                                                                                                                                                                                                                                                                                                                                                                                                                                                                                                                                                                                                                                                                                                                                                                                                                                                                                                                                                                                                                                                                                                                                                                                                                                                                                     |                       |
| 4-amino-N-phenylmorpholine                                                                                                                                                                                                                                                                                                                                                                                                                                                                                                                                                                                                                                                                                                                                                                                                                                                                                                                                                                                                                                                                                                                                                                                                                                                                                                     |                       |
| 1:4-diaminonaphthalene                                                                                                                                                                                                                                                                                                                                                                                                                                                                                                                                                                                                                                                                                                                                                                                                                                                                                                                                                                                                                                                                                                                                                                                                                                                                                                         |                       |
| 4-aminodiethyl-1-naphthylamine                                                                                                                                                                                                                                                                                                                                                                                                                                                                                                                                                                                                                                                                                                                                                                                                                                                                                                                                                                                                                                                                                                                                                                                                                                                                                                 |                       |
| p-aminophenyl-1:4-naphthalenediamine                                                                                                                                                                                                                                                                                                                                                                                                                                                                                                                                                                                                                                                                                                                                                                                                                                                                                                                                                                                                                                                                                                                                                                                                                                                                                           |                       |
| and their water-soluble salts, e. g. chloride, sulfate, acetate, oxalate, etc.                                                                                                                                                                                                                                                                                                                                                                                                                                                                                                                                                                                                                                                                                                                                                                                                                                                                                                                                                                                                                                                                                                                                                                                                                                                 |                       |
| 45. Similarly, other basic compounds which cause the above developing agents to become overall reducing agents may be substituted in whole or in part for the specific bases set forth above. Thus, one or more of the following may be used: Lower alkylamines such as mono-, di- and trimethyl, ethyl, n-propyl, isopropyl, n-butyl, isobutyl, etc. amines, which contain no negative groups, especially hydroxyl groups in the hydrocarbon radicals; straight and branched chain alkyl mono- and poly-amines free from nuclear negative, especially hydroxy groups, e. g. ethylenediamine, tetramethylenediamine, hexamethylene diamine, triaminopropane, $\beta$ -dimethylamino ethylamine, n-propylamylhexylamine, tri-n-amylamine, di-isoamylamine, cyclic and heterocyclic amines, e. g. piperidine, methylpiperidine, ethylpiperidine, piperazine, N-dimethylcyclohexylamine, N - ethyl - N - methyl cyclohexylamine, n-octyl-pyridinium hydroxide; quaternary n-hydroxides free from nuclear substituted negative groups especially hydroxyl groups, e. g. Trimethylbenzylammonium hydroxide Tetramethylammonium hydroxide n - Dodecyldimethylcyclohexylammonium hydroxide n - Dodecyldimethylcyclohexylammonium hydroxide n - Octadecylbenzylidimethylammonium hydroxide n - Dodecylphenyldimethylammonium hydroxide |                       |
| 55. 55.                                                                                                                                                                                                                                                                                                                                                                                                                                                                                                                                                                                                                                                                                                                                                                                                                                                                                                                                                                                                                                                                                                                                                                                                                                                                                                                        |                       |
| 60. 60.                                                                                                                                                                                                                                                                                                                                                                                                                                                                                                                                                                                                                                                                                                                                                                                                                                                                                                                                                                                                                                                                                                                                                                                                                                                                                                                        |                       |
| 65. 65.                                                                                                                                                                                                                                                                                                                                                                                                                                                                                                                                                                                                                                                                                                                                                                                                                                                                                                                                                                                                                                                                                                                                                                                                                                                                                                                        |                       |
| 70. 70.                                                                                                                                                                                                                                                                                                                                                                                                                                                                                                                                                                                                                                                                                                                                                                                                                                                                                                                                                                                                                                                                                                                                                                                                                                                                                                                        |                       |
| 75. 75.                                                                                                                                                                                                                                                                                                                                                                                                                                                                                                                                                                                                                                                                                                                                                                                                                                                                                                                                                                                                                                                                                                                                                                                                                                                                                                                        |                       |

The nitrogenous bases free from negative groups and hydroxyl groups attached to carbon which may be used in practicing this invention are further characterized in that they have an association exponent (pkab) of about 5.00 to about 12.00 and preferably from 9.00 to 11.40.

The proportions of the components of the reducing solutions may be varied considerably. For instance, the amount of arylene-diamino developing agent may vary from 2 to 12 grams per liter with good results. The amount of alkali metal or ammonium sulfite may vary from 5 to 25 grams per liter of solution. The amount of weak alkali, e. g. sodium carbonate may vary from 0 to 30 grams per liter. With regard to the nitrogenous base free from negative groups and hydroxyl groups, it may vary from 8 to 30 grams or ccs. per liter of solution.

Likewise, other color forming compounds may be substituted for the specific ones set forth in the above examples or may be used with any of the herein disclosed arylene diamines. As examples of representative suitable color-formers which are soluble or readily dispersible in the reducing solutions are diacylacetamino-aryl-bis-thiazoles of U. S. Patent 2,140,540, of which difuroylacetamino-1,2,4,5-benzo-bis-thiazole is preferred, the acylacetarylides of U. S. Patent 2,108,602, acetyl acetone, benzoyl acetone, B-naphthoyl acetone, acetoacetic esters, ethyl- $\alpha$ -chloroacetoacetal, ethyl- $\gamma$ -chloroacetoacetate, ethyl malonate, ethyl-p-nitrophenyl-acetate, ethyl propionate, ethyl acetone dicarboxylate, furoylacetic ester, the acylacetamino phenyl morpholines of U. S. Patent 2,133,937, etc.

Suitable magenta color-formers include nitriles, e. g. p-nitrobenzyl cyanide, o-nitro-benzyl-cyanide, p-tolylacetonitrile,  $\omega$ -cyanoacetyl-dibenzfuran,  $\omega$ -cyano-acetyl-acenaphthene, 1- $\omega$ -cyanoacetylcoumarone, 1:3-di-( $\omega$ -cyanoacetyl)-benzene, acyl nitriles, e. g. cyanacetophenone, methoxy- $\alpha$ -naphthoylaceto-nitrile, cyanacetanilides, e. g. 1-cyanacetamino-benzthiazole, etc., pyrazolones, e. g. 1-phenyl-3-furyl-5-pyrazolone, 1-phenyl-3-carboxylic acid-5-pyrazolone, 1-phenyl-3-hydroxy-5-imino-pyrazolone, 1-(8'-quinolyl)-3-methyl-5-pyrazolone, 1-phenyl-3-methyl-5-thiopyrazolone, etc.

Suitable blue-green color formers include phenols, e. g. ortho and meta-chlorophenol, o-bromophenol, o-iodophenol; naphthols, e. g. 2,3,4-trichloronaphthols, 2,6-dibromo-1,5-dihydroxy naphthalene, etc.

An important advantage of the present invention resides in the fact that the readily available weak arylene diamino types of developing agents may readily be converted into powerful reducing agents in a simple manner and with the aid of inexpensive and readily available additional agents.

A further advantage resides in the fact that a weak developing agent of the arylene diamine type becomes readily converted into an excellent color developing agent producing a much greater dye density for the same amount of reduced silver by the addition of inexpensive and readily available photographic materials.

Any suitable developers of the type used as the first developer in a reversal process can be used for the development of the negative images. An energetic working developer is preferably used to give full detail and harmonious color rendering. It is also desirable that the developer selected produce a minimum of relief effect in the gelatin. To this end, caustic alkalies should

be avoided. Sodium carbonate is preferable as an alkali and is used in smaller amounts than generally used in reversal "first developers." "Metol" in combination with hydroquinone, for instance, is suitable as the developing agent, as are also acid amidol developers where the films do not contain color-formers. The development at this stage should be carried out completely, that is none of the latent images should be left undeveloped.

A suitable developer for the above purpose is

*Developer A*

|                         |       |      |
|-------------------------|-------|------|
| Metol                   | grams | 2.5  |
| 15 Hydroquinone         | do    | 9.0  |
| Sodium sulfite, anhy.   | do    | 75.0 |
| Sodium carbonate, anhy. | do    | 50.0 |
| Potassium bromide       | do    | 3.5  |
| Water to                | liter | 1    |

20 A number of steps required in reversal development processes are eliminated by this invention which is of major importance. The elimination of one or more steps means that a shorter processing time is required. A more simplified 25 continuous developing machine may be used. A substantial savings of chemicals, wash water costs, etc. is effected.

The present invention provides an improvement over previous suggestions for reversal development, wherein residual silver halides are chemically exposed by means of sulfur bearing compounds such as thiourea, allyl thiourea, etc. since these proposals incur the need for additional tubes or tanks in processing machines, more wash water consumption and an extended 35 total processing time. Furthermore, such compounds are undesirable because of their objectionable odor.

30 40 A further advantage resides in the fact that a much greater density of dye image is produced with the same silver density as compared with the usual color developers containing alkaline carbonates as pH regulators.

An additional advantage resides in the fact 45 that a very great increase in the coupling velocity of color formers is obtained by the use of the baths containing arylene diamino compounds and certain nitrogenous bases as energizers. Still other advantages will be apparent to those skilled 50 in the art.

As many apparently widely different embodiments of this invention may be made without departing from the spirit and scope thereof, it is to be understood that the invention is not limited 55 to the specific embodiments hereof except as defined in the appended claims.

I claim:

1. A photographic reversal process comprising developing a photographic element containing a 60 latent image in an ordinary developer to produce a negative image and developing the reversed image without re-exposure in the presence of a color former with an aqueous reducing bath containing a compound of the general formula:



70 wherein R and R' are members of the group consisting of hydrogen and alkyl radicals of 1 to 4 carbon atoms, and the water soluble salts thereof, and an aliphatic amine of 1 to 6 carbon atoms in an amount sufficient to change the characteristics of the solution so that it no longer

distinguishes between exposed and unexposed silver salts, said amount being within the range from 8 ccs. to 30 grams per liter of solution.

2. A process as set forth in claim 1 wherein the photographic element contains non-migratory color formers in the emulsion layers.

3. A photographic reversal process which comprises developing a photographic element containing a latent image in an ordinary developer to produce a negative image and developing the reversal image without re-exposure in the presence of a color former with an aqueous reducing bath containing an aromatic primary amino developing agent and an aliphatic amine of 1-6 carbon atoms in an amount sufficient to change the characteristics of the solution so that it no longer distinguishes between exposed and unexposed silver salts, said amount being within the range from 8 ccs. to 30 grams per liter of solution.

4. A process as set forth in claim 3 wherein said amine is hexamethylenediamine.

5. A photographic reversal process which comprises developing a multilayer film having three

10 differentially sensitized emulsion layers superimposed on a transparent base, said layers containing an immobile color former capable of forming a dye upon color forming development 5 complementary in color to the sensitivity of the respective layers, which has been exposed to a colored object, in an ordinary developer to produce silver color-component images in the respective layers and simultaneously developing the reversed images without re-exposure in an aqueous reducing bath containing as the sole type of reducing agent an aromatic amino developing agent having an unsubstituted amino group and an aliphatic primary amine of 1 to 6 carbon atoms in 15 an amount sufficient to change the characteristics of the solution so that it no longer distinguishes between exposed and unexposed silver salts, said amount being within the range from 8 ccs. to 30 grams per liter of solution.

20 6. A process as set forth in claim 5 wherein said amine is hexamethylenediamine.

7. A process as set forth in claim 5 wherein said amine is hexamethylenediamine.

EMERY MESCHTER.

CERTIFICATE OF CORRECTION.

Patent No. 2,310,981.

February 16, 1943.

EMERY MESCHTER.

It is hereby certified that error appears in the printed specification of the above numbered patent requiring correction as follows: Page 5, second column, line 29, for the patent number "2,182,184" read --2,182,814--; page 6, first column, line 8, for "2,195,149" read --2,195,419--; line 45, for "wellow" read --yellow--; and that the said Letters Patent should be read with this correction therein that the same may conform to the record of the case in the Patent Office.

Signed and sealed this 20th day of April, A. D. 1943.

Henry Van Arsdale,

Acting Commissioner of Patents.

(Seal)